

# UNITED STATES PATENT OFFICE.

JOHN H. RYAN, OF PORTLAND, OREGON.

## PROCESS OF TREATING ORES.

No. 841,721.

Specification of Letters Patent.

Patented Jan. 22, 1907.

Application filed March 1, 1906. Serial No. 303,664.

*To all whom it may concern:*

Be it known that I, JOHN H. RYAN, a citizen of the United States, residing at Portland, in the county of Multnomah and State of Oregon, have invented certain new and useful Improvements in Processes of Treating Ores, of which the following is a specification.

This invention is a process of treating ores, and is more particularly adapted for the treatment of such ores as contain metals yielding soluble sulfates or sulfites, often containing also the precious metals. Of such ores those containing copper, or copper and nickel, or nickel and cobalt, or cobalt, may be considered as types.

Such ores generally occur in combination with sulfur or arsenic, and if they are subjected to a roasting operation of the usual character there results not only a loss of a portion of the precious metals, but the copper, nickel, and cobalt are transformed into such difficultly-soluble compounds that a very imperfect extraction is afforded when they are subsequently leached.

I have discovered that by proceeding in a definite manner as hereinafter set forth the extraction of the metal values and their recovery may be effected with substantially quantitative results.

The preliminary treatment is substantially the same in all cases. The ore is crushed and then ground to pass a standard screen of sixty to one hundred and twenty mesh—that is, the ore is ground to such degree of fineness as is usually employed in preparation for leaching. The fine ore is spread upon the hearth of a muffle-roaster and constantly agitated thereon and is maintained at a temperature not exceeding 300° Fahrenheit for a definite period, usually about one hour, until reaction has substantially ceased. It is then further heated to a temperature not exceeding 450° Fahrenheit, this temperature being likewise maintained for about the same period with constant rabbling of the ore. The temperature is then again increased and is maintained at 800° Fahrenheit or less for a further period of about one hour, when it is raised to approximately 1,000° Fahrenheit, this temperature, corresponding to a red-heat, being maintained for about an hour or until the volatile impurities are entirely eliminated. The ore is then discharged while still hot into a suitably dilute solution of sulfuric or sulfurous acid for the preparation of the sulfate or sulfite solution.

Such acid solution is preferably prepared from the gases derived from the roasting in known manner.

I do not desire to restrict myself to the number of successive heating stages above mentioned nor to any precise degree of temperature nor period of time for the several stages, for, as will be understood, the conditions are subject to some variation in accordance with the character of the ore. I have found it essential, however, to the best results that the roasting should occur in successive stages and that the temperature should be maintained approximately constant during each of said stages. I have also found it to be desirable that during each stage the temperature should be maintained until the volatilization or separation of impurities has substantially ceased. As above stated, the metals after such treatment are found to be soluble in the acid solvents used to a degree not otherwise attainable.

I do not limit myself to any particular form of roaster; but I have found a roasting-furnace of the McDougall type well suited to my purpose. In the use of this roaster in accordance with my process a pyrometer is provided in connection with each of the shelves, and the ore is rabbled under constant temperature conditions maintained by manipulation of hot and cold air inlets for a definite time before being transferred to the shelf below, where the treatment is continued at a suitable higher temperature. In this manner the ore is transferred from shelf to shelf and rabbled at progressively-increasing temperature and is finally discharged into the leaching-vat.

In the case of ores containing nickel or cobalt it is advantageous to add to the ores before conveying the same to the roasting-furnace about 2--3 per cent. of sodium chlorid. The roasting is conducted with the same precautions as above described, and the subsequent leaching is effected with the same solvents. The leaching is preferably effected in a continuous manner, the solvent being circulated successively through the leaching-tank and through a suitable precipitating apparatus for the metal. The initial temperature of the leaching solutions should be not less than 150° Fahrenheit, and where electrolytic precipitation is employed as herein described the deposition should be effected at a temperature not below 80° Fahrenheit. After the metals yielding soluble sulfates or

sulfites are extracted the tailings are treated for the recovery of precious metals, if such be present. For this purpose they are neutralized by lime or by the hydroxid or carbonate of sodium or potassium and are then subjected to the solvent action of a cyanid or other solution, the gold and silver being recovered in the usual manner.

In some cases, and more particularly when 10 treating cobalt ores containing gold and silver, I find it advantageous to regrind the tailings wet, as the precious metals are then more readily and completely dissolved.

The treatment of the metal-bearing solutions obtained by leaching must be varied somewhat in accordance with the character of the ore. For copper ores the copper is preferably electrodeposited in a continuous depositing-tank, using insoluble anodes, the 15 tank being preferably of the character described in my copending application, Serial No. 303,663, filed March 1, 1906.

In case iron is present in the ores it passes 20 into the solution, the iron salts being oxidized in the region of the insoluble anodes. Such salts when returned to the leaching-vat become effective solvents for the compounds of copper. When both copper and nickel are present, I prefer to precipitate the copper as 25 sulfid and then to separate the nickel by electrolysis with insoluble anodes, the copper sulfid being either redissolved and the metal electrodeposited or else reduced to metal, cast into anodes, and electrolytically refined.

30 In case nickel and cobalt are present together in solution I may add an alkali hydroxid in quantity just sufficient for the precipitation of the nickel, thereafter electrodepositing the cobalt from the clear solution. The nickel 35 may be recovered in any suitable manner, as by solution of the hydroxid and electrodeposition of the metal or by conversion of the same into metal anodes suitable for electrolytic refining.

40 In the case of ores containing copper and nickel the iron is generally present as magnetic oxid, and after the copper and nickel have been leached out the tailings may be dried, reground, and passed through a magnetic separator for the recovery of the iron. 45 The pure magnetic oxid so obtained may be

subsequently smelted, preferably utilizing the electric power where available.

I claim—

1. The process of treating ore preparatory 55 to leaching which consists in roasting the ore in successive stages at progressively higher temperatures, the ore being heated at each stage for an optional time, and maintaining it in agitation throughout the roasting operation, substantially as described.

2. The process of treating ore preparatory to leaching which consists in reducing the ore to a fine state of division, then roasting the ore in successive stages at progressively 60 higher temperatures, the ore being heated at each stage for an optional time, and maintaining it in agitation throughout the roasting operation, substantially as described.

3. The process of treating ore preparatory 65 to leaching which consists in mixing therewith sodium chlorid, and then roasting the ore in successive stages at progressively higher temperatures, the ore being heated at each stage for an optional time, substantially 70 as described.

4. The process of treating ore containing nickel or cobalt preparatory to leaching which consists in mixing therewith sodium chlorid, then roasting the ore in successive 75 stages at progressively higher temperatures, the ore being heated at each stage for an optional time, and maintaining the ore in agitation throughout the roasting operation, substantially as described.

5. The process of treating sulfid ore which 80 consists in grinding the ore to the degree of fineness requisite for leaching, then roasting the ore in successive stages at progressively higher temperatures, the ore being heated at 85 each stage for an optional time, maintaining the ore in agitation throughout the roasting operation, converting the roaster-gases into a solvent solution, and discharging the roasted ore while still in a heated state into the solution so prepared, substantially as described.

In testimony whereof I affix my signature in presence of two witnesses.

JOHN H. RYAN.

Witnesses:

C. W. FOWLER,  
J. B. HILL.